

M. ARENDT.

DEPOSITING REPAIR METAL ACROSS AN ALTERNATING CURRENT ARC.

APPLICATION FILED OCT. 23, 1914.

1,146,988.

Patented July 20, 1915.



WITNESSES:

K. Schuly.  
L. Bates

INVENTOR

Morton Arendt

BY

Lewis Davis Goldsbrough  
ATTORNEYS

# UNITED STATES PATENT OFFICE.

MORTON ARENDT, OF NEW YORK, N. Y., ASSIGNOR TO HEINRICH L. J. SIEMUND, OF NEW YORK, N. Y.

## DEPOSITING REPAIR METAL ACROSS AN ALTERNATING-CURRENT ARC.

1,146,988.

Specification of Letters Patent.

Patented July 20, 1915.

Application filed October 23, 1914. Serial No. 868,162.

*To all whom it may concern:*

Be it known that I, MORTON ARENDT, a citizen of the United States, residing in the city, county, and State of New York, have invented certain new and useful Improvements in Depositing Repair Metal Across an Alternating-Current Arc; and I do hereby declare the following to be a full, clear, and exact description of the invention, such as will enable others skilled in the art to which it appertains to make and use the same.

In recent years extensive use has been made of the process of repairing boilers, and such other articles as are inaccessible and cannot readily be handled, by the deposition of repair metal across a direct current arc playing between the metal to be repaired and the tip of a small electrode of the repair metal. In that process considerable difficulty is experienced in striking the arc and maintaining it without interruption, and some degree of experience and skill is necessary to the successful carrying out of the operation. The arc will not be maintained until the spot on the metal to be repaired has been well heated by the electrical energy expended at the point of contact. After the arc is struck it is maintained at a length of about  $\frac{1}{8}$  of an inch by skilful manipulation on the part of the operator, and if it is drawn out much beyond that length the accompanying decrease in current, due to the increase of the resistance, tends to extinguish the arc. The desirable conditions are, first, provision for developing the required heating energy at the point of contact, and second, means for maintaining the current value as nearly constant as possible—that is, means for reducing the current variations due to slight alterations of the length of the arc. It is for this latter reason that a steady resistance is always inserted in the direct current circuit, in series with the electrode. I have discovered that these desirable conditions may be more fully attained by a novel arrangement of alternating current circuit containing a properly proportioned inductance, in accordance with the following disclosure, and this discovery is the more remarkable in view of the fact that it has heretofore been supposed that alternating current is unsuitable for

carrying on this process of deposition of repair metal across the arc, so that it has heretofore been the practice, and the recommendation of those skilled in the art, to use a motor-generator for transforming the alternating current into direct current, whenever a direct current supply is not immediately available. It is in fact true that if the circuit connections and voltages commonly employed with direct current are used for alternating current work, the time required to properly heat the surface of the work, where the repair metal is to be deposited, is almost prohibitive. The welder is constantly trying to strike the arc which just as regularly goes out and as a result only globules of the electrode metal are deposited on the work surface, and no homogeneous union is made.

I have discovered that by making use of a relatively high initial voltage and inserting a properly proportioned inductance in series with the arc, I can produce the desired conditions (a good initial heating energy, and the maintenance of substantially constant current), to an improved degree, so that the arc may readily be struck and will be maintained, even though the operator varies the length of the arc to a greater extent than has heretofore been possible. It will readily be understood that this increases the facility of the operation not only at its start but throughout, because movements of the hand of the operator which would heretofore extinguish the arc, may now occur without extinguishing it. Furthermore, I find that under these conditions, deposition of the repair metal, either on the flat or against gravity, may readily be practised with an economy of energy as compared with direct current practice. In fact, only about 60 to 70 per cent. as much energy is required, while a great advantage obtains from the elimination of motor generator sets and the substitution of a simple low cost static transformer; and this saving is accompanied by an increase, rather than a decrease, in the strength of the weld.

In the accompanying diagrammatic drawing I have illustrated a suitable system.

In this diagram 1 is the article to be repaired; 2 is the repair electrode; 3 is an alternating current source here shown as the

secondary of the transformer 4, fed from the mains 5, 6; although it will be understood that any other suitable source of alternating current may be employed.

5 7 is the inductance which is to be proportioned in the manner hereinafter described, and 8 is an adjustable resistance.

I have found that the best conditions for effective welding with this system, when working on heavy metal structures, such as 10 steam boilers, piping, locomotive fittings and the like, employing iron or steel wire electrodes of from 0.12 inch to 0.19 inch in diameter, results when the voltage applied to the welding circuit is about 110 to 120 volts and the current from 150 to 180 amperes, and the voltage drop across the terminals of the inductance, that is, the inductive voltage component, is between 75 and 15 105 volts, and the total resistance drop of the system is between 10 and 40 volts, the general rule being that the most economical conditions obtain with the higher inductance and lower resistance drops. For the purpose of attaining the desired resistance drop I 20 may include the adjustable resistance 8 in the circuit or the resistance drop may reside in the leads and the other elements of the circuit. With this described arrangement 30 the power required for proper deposition of the metal to form a homogeneous part of the work to be repaired, is only from  $6\frac{1}{2}$  to  $7\frac{1}{2}$  kilowatts at about 110-120 volts, while for corresponding results with direct current 10 $\frac{1}{2}$  to 14 kilowatts, that is 150 to 200 amperes at 35 70 volts, are regularly employed. It will be understood that the inductance 7 may reside in the transformer itself, as by using a transformer in which the magnetic leakage is exaggerated.

40 If thin metal sheets are to be joined or added to by deposition from the metallic electrodes, the current should be reduced in value by increasing the impedance of the circuit, and the electrodes may also be reduced in diameter where necessary.

With the above conditions I find that not only is the welding arc readily struck and maintained, but the welding surface is 50 promptly brought to the proper temperature, that is, to such a temperature that the surface becomes incipiently fused or heated to such a degree that the deposited metal will combine therewith homogeneously. This 55 result is secured whether the work being repaired is placed above or below the electrode, and whether the electrode clamp is provided with a magnetizing coil or not, and whether or not welding powder or flux coatings are used on the electrodes, though the presence of the latter seems to reduce to 60 some extent the amount of dripping when the metal is to be deposited against gravity. The use, however, of these auxiliaries, 65 namely, the magnetizing coil and flux coat-

ings, is well known in the art and does not form any part of my discovery.

Using the high inductance and low resistance referred to, I have uniformly made welds having a strength of 46,000 pounds 70 per square inch, somewhat beyond the elastic limit of the structures united by the deposited metal. The break is crystalline in appearance and shows no slag. The weld with a somewhat smaller inductance and 75 slightly greater resistance has substantially the same strength averaging about 44,000 pounds, but the power required is greater, about 9.5 to 10.5 kilowatts, though still slightly less than with direct current. In 80 any case, however, the inductive voltage component should substantially exceed the voltage drop across the arc.

The drop across the arc will ordinarily 85 vary from about 22 volts to about 30 volts, depending upon the length of the arc. This is a greater variation than can be tolerated in direct current work, but I find that even greater variations can accompany successful welding with my system. In fact, I have 90 successfully welded with the arc voltage varying from 15 to 35 volts.

I have commonly employed a frequency of sixty cycles per second in my work. In general a higher frequency facilitates the 95 work, while lower frequencies tend to make it more difficult. If the available frequency is too low a static frequency transformer may be used.

#### What I claim is:

1. A system for building up upon a metal surface a homogeneous deposit of repair metal, comprising an electrode of the repair metal connected in an electric circuit with the metal to be repaired, so that an electric 100 arc may be drawn between them, said circuit including a source of alternating current and having inductance of such value that the inductive voltage component substantially exceeds the voltage drop across the 105 arc.

2. A system for building up upon a metal surface a homogeneous deposit of repair metal, comprising an electrode of the repair metal connected in an electric circuit with the metal to be repaired, so that an electric 110 arc may be drawn between them, a source of alternating electro-motive force in said circuit having a voltage of approximately from 110 to 120 volts, and said circuit having inductance of such value that the inductive voltage component is from 75 to 105 volts.

3. A system for building up upon a metal surface a homogeneous deposit of repair metal, comprising an electrode for the repair metal connected in an electric circuit with the metal to be repaired, so that an electric 120 arc may be drawn between them, a source of alternating electro-motive force in said circuit having a voltage of approximately from 125 130

110 to 120 volts, and said circuit having inductance of such value that the inductive voltage component is from 75 to 105 volts, and ohmic resistance of such value that the 5 resistance drop is approximately 10 to 40 volts.

In testimony whereof I affix my signature, in presence of two witnesses.

MORTON ARENDT.

Witnesses:

KENNETH P. PENNIE,  
M. A. BILL.